

Patented Feb. 15, 1927.

1,618,029

# UNITED STATES PATENT OFFICE.

SRINIVAS RAM WAGEL, OF NEW YORK, N. Y., ASSIGNOR TO THE LEHIGH COAL AND NAVIGATION COMPANY, A CORPORATION OF PENNSYLVANIA.

## PROCESS FOR BRIQUETTING COAL.

No Drawing.

Application filed September 30, 1924. Serial No. 740,839.

This invention relates to a process for briquetting coal, the present application being a continuation in part of my copending application, Serial No. 708,571, filed April 5, 1924.

More specifically the invention relates to a process which includes the use, in a briquette bonded by clay, of ingredients in the binder which will remain sufficiently adhesive, up to the temperature at which the clay becomes baked, to adequately perform the binding function.

Heretofore much difficulty has been experienced in selecting a suitable binder for fine sizes of coal in the manufacture of coal briquettes. It is essential that a briquette burn with but little smoke and without odor, that it will withstand reasonably high temperatures without disintegrating or becoming sticky and losing its shape, and that it will withstand the action of water without deterioration. In other words, it is necessary to provide a binder for fine coal which will not interfere with the burning of the coal, and which will not produce a great amount of ash, but which will resist the action of water and retain its shape under pressure and heat.

In order to sufficiently harden the well-known clay binder of a briquette it is necessary to raise the temperature of the briquette to from 600° to 700° Fahrenheit. The briquette is preferably baked to harden the binder, such baking requiring a temperature of from 800° to 1000° Fahrenheit, or something under the ignition point of the coal during the short period of baking.

Where asphalt, or other bituminous binders such as heavy oils or coal tar, are used however, the binding quality is lessened or lost entirely at a temperature of about 400° Fahrenheit, or even lower, resulting in a disintegration of the briquette before its ignition point is reached.

It is a primary object of the present invention to prevent disintegration of a coal briquette within ordinary ranges of temperature, and before its ignition point is reached, by combining with a clay binder ingredients which will retain adhesive qualities up to a temperature at which the clay becomes baked, to adequately perform the binding function.

A further object is to produce a briquette which is substantially impervious to mois-

ture, which burns with but little smoke and ash, which possesses great resistance to crushing stress, and which will not soften or disintegrate within ordinary ranges of temperature.

These objects, together with others which will be apparent as the description proceeds, are accomplished as follows:

The process broadly contemplates the use of a binder composed of clay and sulphite liquor, molasses, alcohol slops, meaning molasses after alcohol is extracted therefrom, magnesium chloride, or the like, with a bituminous substance such as asphalt or coal tar, blended and stabilized by the addition of an acid or a mixture of acid and oil, all thoroughly mixed with fine coal and hardened in the form of a briquette.

Sulphite liquor, molasses, alcohol slops, and magnesium chloride are typical substances which will retain their adhesive qualities between 400° and 800° Fahrenheit. Any one of these, when mixed with clay as a binder for fine coal, will retain the shape of the moulded briquette until the clay bakes or hardens sufficiently for this purpose. In the case of asphalt or bituminous substances such as coal tar and so forth, the binding power would be lost at about 400° Fahrenheit, thereby leaving no adequate binding agent at temperatures of from 400° to 600° and 700° Fahrenheit.

It is preferable that the briquette be baked, for by baking it is made more water-resistant and mechanically stronger. The briquettes are more satisfactorily hardened if the baking is carried on in a more or less oxidizing atmosphere as contrasted to a closed oven or the like.

It is essential that the binder have bituminous ingredients, such as asphalt or heavy oil, or possibly coal tar, for several purposes, among others to supply fixed carbon to the baked briquette to render it waterproof, as well as to act as an initial binder at temperatures below 400° Fahrenheit. Sulphite liquor, molasses, alcohol slops, or magnesium chloride alone would not leave enough fixed carbon to render the briquette satisfactorily waterproof, and sulphite liquor is not alone a good binder during the process of baking under oxidizing conditions. Accordingly, the bituminous substance supplies both deficiencies.

In the process of baking the briquette is

first passed through regions of gradually increasing heat, such regions being alternated by regions of cooling. The moisture is first drawn off at low temperatures, then the volatile constituents of asphalt or other bitumen such as heavy oil, coal tar, or other pitchy materials, go off up to temperatures of about 400° Fahrenheit, leaving a substantial percentage of fixed carbon, and at about 600° 10 Fahrenheit the clay begins to bake sufficiently to act as a permanent binder. When the briquette is passed through that region of the oven, the temperature of which is approximately 800° Fahrenheit, the volatile constituents of the sulphite liquor, molasses, alcohol slops, magnesium chloride or the like, have been nearly all driven off leaving mostly ash as the residue of the temporary binder.

As a blending and stabilizing agent acids 20 used alone or in combination with oils, may be added to the binder.

A specific example of the use of my process with sulphite liquor, which is at present a cheap substance possessing the necessary qualities of a temporary binder to prevent disintegration of a briquette between the temperatures of 400° and 800° Fahrenheit, is as follows:—

About 40 parts of concentrated sulphite 30 water liquor, containing 50% water, is thoroughly mixed with about 13 parts of clay and about 18 parts of water in a steam-jacketed agitator of the type in common use. It is here brought to a temperature of 35 from 170° to 190° Fahrenheit, the agitation being continued during such heating. Upon reaching the desired temperature, 1 to 2 parts of a liquid composed of equal parts of sulphuric acid and Panuco oil of 12 to 16° 40 Baumé is added and agitation continued. Panuco oil is a petroleum of asphalt base, produced in the Panuco district of Mexico. It is generally heavy, or of low Baumé gravity, and contains from 2 to 5% sulphur. The 45 solid matter resulting from the mixture of Panuco and sulphuric acid is separated from the liquid and the liquid only is used in this step of the process.

Next, approximately 27 to 33 parts of asphalt or other bituminous material is added, the bitumen having been previously heated to a temperature of from 225° to 275° F. in which condition it will readily flow. Asphalt, for use as a binder should possess a 55 fair degree of ductility, and should have a melting point of from 110° to 170° Fahrenheit.

Agitation of the entire mixture is continued during the addition of the bitumen, and 60 preferably continued for approximately thirty minutes thereafter.

As an alternative to the process described above, this invention further contemplates the mixing of the asphalt or other bituminous material with the solution of sulphite

liquor, clay and water, simultaneously, rather than in pouring the bitumen into the sulphite liquor, clay and water solution as previously described.

As a further alternative, the total amount of water need not be added at the time of the mixture of the sulphite liquor and clay as set forth above, but from 8% to 10% water may be added in the initial step of the process, and the remainder introduced after the bitumen has been added to the mixture.

The resulting composition is the binder which is mixed with fine coal in the proportions of from one part binder to twenty parts of coal, to one part binder for ten parts of coal.

The briquette so made is far from being impervious to moisture. To make it so, it is subjected to a heating or baking process, during which the volatile constituents of the asphalt or other bitumen go off up to temperatures of about 400° Fahrenheit, leaving a fair percentage of fixed carbon. At about 600° or 700° Fahrenheit the clay begins to bake sufficiently to act as a final or permanent binder. As hereinbefore pointed out the baking should take place in a more or less oxidizing atmosphere.

In order to properly bake the briquette it has been found essential to pass it through a series of regions of gradually increasing heats, ranging from about 250° Fahrenheit to about 1000° Fahrenheit as a maximum. These regions of increasing heat are alternated by regions through which the briquette passes to be cooled somewhat before entering the next region of high temperature. This serves to alternately expand and contract the briquette composition, thereby knitting the constituents thereof more closely and increasing the strength of the resulting product.

An apparatus for baking the briquettes as set forth is described more in detail in my copending application, Serial No. 709,181, filed April 26, 1924.

The product resulting from the above process is a hard and compact mass which possesses great resistance to pressure and which is substantially waterproof, but which burns with little smoke and odor, and leaves but a small amount of ash.

What I claim as my invention is:—

1. A briquette comprising coal bonded by clay, bituminous material, and a binding agent effective to adequately bind the briquette together at temperature ranges between the point where the bituminous material loses its binding qualities and the clay becomes sufficiently baked to hold the briquette against disintegration.

2. A briquette comprising coal bonded by clay, bituminous material, and a binding agent effective to adequately bind the briquette together at temperature ranges be-

tween the point where the bituminous material loses its binding qualities and the clay becomes sufficiently baked to hold the briquette against disintegration, wherein the 5 briquette is heated sufficiently to bake the clay as aforesaid.

3. In the manufacture of coal briquettes the process which comprises preparing an aqueous suspension of clay, mixing there- 10 with additional binding matter effective to adequately bind the briquette together at temperature ranges up to a temperature at which the clay will be sufficiently baked to hold a briquette against disintegration, and 15 briquetting coal therewith.

4. The process of claim 3, with the additional step of heating the briquettes so formed to a temperature sufficient to bake the clay as aforesaid.

20 5. In the manufacture of coal briquettes, the process which comprises mixing together bituminous material, an aqueous suspension of clay, and a binding agent effective to adequately bind a briquette together at temperature 25 ranges between the point where a bituminous material loses its binding power and the clay becomes sufficiently baked to hold a briquette against disintegration, and briquetting coal therewith.

30 6. The process of claim 5, together with the additional step of heating the briquette to a temperature sufficient to bake the clay as aforesaid.

7. In the manufacture of coal briquettes, 35 the process which comprises mixing an acid together with a bituminous material, an aqueous suspension of clay, and a binding agent effective to adequately bind a briquette together at temperature ranges between the 40 point where bituminous material loses its binding power and the clay becomes sufficiently baked to hold a briquette against disintegration, and briquetting coal therewith.

45 8. In the manufacture of coal briquettes, the process which comprises binding fine coal by a mixture of asphalt, clay, and sulphite liquor.

9. In the manufacture of coal briquettes, 50 the process which comprises binding fine coal by a mixture of asphalt, clay, and acidulated sulphite liquor.

10. In the manufacture of coal briquettes, 55 the process which comprises preparing a solution of sulphite water liquor, clay and water; in agitating such solution and gradually heating it; in adding a small quantity of acidified oil during agitation of the solution; in adding heated asphalt during such 60 agitation, and in finally mixing the binder so prepared with fine coal.

11. In the manufacture of coal briquettes, 65 the process which comprises preparing a suspension of clay in a solution of sulphite liquor; adding acidified oil thereto as a

blending and stabilizing agent; introducing asphalt into the solution; briquetting the coal therewith, and finally in heating the coal briquette to harden the clay.

12. In the manufacture of coal briquettes, 70 the process which comprises preparing a solution of sulphite water liquor, clay, and water; in heating and agitating such solution; in heating asphalt; in mixing the heated asphalt with the solution previously 75 prepared; in agitating the mixture so made; and in finally adding fine coal thereto.

13. In the manufacture of coal briquettes, 80 the process which comprises preparing a solution of sulphite liquor and clay with a small amount of water; in heating and agitating the solution; in adding acidified oil to such solution; in inducing heated asphalt into the mixture; in adding water; in agitating the mixture, and in finally adding 85 fine coal to such mixture.

14. In the manufacture of coal briquettes, 90 the process which consists in preparing a solution of sulphite water liquor, clay, and water; in agitating such solution, and in adding acidulated oil thereto; in gradually heating the solution while agitating; in adding heated asphalt to the solution during such agitation, and in continuing agitation 95 thereafter; in mixing predetermined quantities of the composition so formed with fine coal, moulding said composition in the form of briquettes, allowing the moisture to drain from the briquettes so formed, passing the unfinished briquettes through regions which 100 heat them to successively higher temperatures, and in partially cooling such briquettes between each heating operation.

15. As an article of manufacture, a coal 105 briquette composed of fine coal with a binder of asphalt, sulphite liquor, and clay, baked to be substantially waterproof.

16. In the manufacture of coal briquettes, 110 the process which comprises binding coal particles into briquette form by a bituminous binder; baking the briquettes by passing them successively through regions which heat them to progressively higher temperatures and cooling them between successive heatings.

17. In the manufacture of coal briquettes, 115 the process which comprises binding coal particles into briquette form by clay and a bituminous binder, and baking the briquettes 120 by passing them successively through regions which heat them to progressively higher temperatures.

18. In the manufacture of coal briquettes, 125 the process which comprises binding coal particles into briquette form by a binder of clay, bituminous material, and a further binding agent, effective to adequately bind the briquette together at temperature ranges between the point where the bituminous material loses its binding power and the clay 130

becomes sufficiently baked to hold the briquette against disintegration; baking the briquettes by passing them successively through regions which heat them to progressively higher temperatures, and cooling them between successive heatings.

19. In the manufacture of coal briquettes, the process which comprises binding coal particles into briquette form by a binder of clay and additional material effective to adequately bind the briquette at temperature ranges up to a temperature at which the clay will be baked sufficiently to hold the briquettes against disintegration; baking the briquettes by passing them successively through regions which heat them to progressively higher temperatures, and cooling them between successive heatings.

20. In the manufacture of coal briquettes, the process which comprises preparing a solution of sulphite water liquor, clay and water; in agitating such solution and gradually heating it; in adding a small quantity of acid during agitation of the solution; in adding heated asphalt during such agitation; and in finally mixing the binder so prepared with fine coal.

21. In the manufacture of coal briquettes, the process which comprises preparing a suspension of clay in a solution of sulphite liquor; in adding acid thereto as a blending and stabilizing agent; introducing asphalt into the solution; briquetting coal therewith; and finally in heating the coal briquettes to harden the clay.

22. In the manufacture of coal briquettes, the process which comprises preparing a solution of sulphite liquor and clay in a small amount of water; in heating and agitating the solution; in adding acid thereto; in inducing heated asphalt into the mixture; in adding water; in agitating the mixture; and in finally adding fine coal to such mixture.

23. In the manufacture of coal briquettes, the process which consists in preparing a solution of sulphite water liquor, clay, and water; in agitating such solution; and in adding acid thereto; in gradually heating the solution while agitating; in adding heat-

ed asphalt to the solution during such agitation, and in continuing agitation thereafter; in mixing predetermined quantities of the composition so formed with fine coal; moulding said composition in the form of briquettes; allowing the moisture to drain from the briquettes so formed; passing the unfinished briquettes through regions which heat them to successively higher temperatures; and in partially cooling such briquettes between each heating operation.

24. A briquette comprising coal bonded by clay and additional binding material effective to adequately bind the briquette at temperature ranges up to a temperature at which the clay will be baked sufficiently to hold the briquette against disintegration.

25. A briquette comprising coal bonded by clay and additional binding material effective to adequately bind the briquette at temperature ranges up to a temperature at which the clay will be baked sufficiently to hold the briquette against disintegration, said briquette having been sufficiently heated to bake the clay as aforesaid.

26. In the manufacture of coal briquettes, the process which comprises mixing coal particles and a binder, briquetting the mixture and passing the briquettes successively through a plurality of hot zones and through substantially cooler zones interposed between certain of the hot zones, whereby the briquettes are alternately subjected to heating and cooling to expand and contract the same.

27. In the manufacture of coal briquettes, the process which comprises mixing coal particles and a binder, briquetting the mixture and passing the briquettes successively through zones heated to graduated temperatures up to about 1,000° F. and also passing the briquettes through zones at substantially lower temperatures between certain of said hot zones, whereby the briquettes are alternately subjected to heating and cooling to expand and contract the same.

In testimony whereof I affix my signature.

SRINIVAS RAM WAGEL